

# United States Patent [19]

Krause

[11] 4,175,967

[45] Nov. 27, 1979

[54] Multipart photosensitive element with independent contrast control of constituent part records

[76] Inventor: Donald Krause, 5 Old Towne Rd., Apt. #236, Ayer, Mass. 01432

[21] Appl. No.: 847,583

[22] Filed: Nov. 1, 1977

[51] Int. Cl.<sup>2</sup> ..... G03C 1/76; G03C 3/00

[52] U.S. Cl. ..... 430/503; 430/509

[58] Field of Search ..... 96/68, 69

## [56] References Cited

### U.S. PATENT DOCUMENTS

|           |         |               |       |
|-----------|---------|---------------|-------|
| 3,141,773 | 7/1964  | Hellmig       | 96/68 |
| 3,450,536 | 6/1969  | Wyckoff       | 96/68 |
| 3,637,388 | 1/1972  | Ranz          | 96/69 |
| 3,663,228 | 5/1972  | Wyckoff       | 96/69 |
| 3,672,898 | 6/1972  | Schwan et al. | 96/68 |
| 3,776,733 | 12/1973 | Lohmer et al. | 96/68 |
| 3,798,037 | 3/1974  | Silverman     | 96/59 |

|           |         |             |       |
|-----------|---------|-------------|-------|
| 3,849,138 | 11/1974 | Wyckoff     | 96/68 |
| 3,941,595 | 3/1976  | Ranz et al. | 96/68 |
| 3,977,872 | 8/1976  | Hellmig     | 96/69 |
| 3,992,210 | 11/1976 | Evans       | 96/69 |
| 4,003,744 | 1/1977  | Kliem       | 96/74 |

Primary Examiner—Mary F. Kelley  
Attorney, Agent, or Firm—Joseph S. Iandorio

## [57] ABSTRACT

A multipart photosensitive element having a predetermined saturation density including at least two partial record portions for forming a full record, each partial record portion controlling a preselected density range of the full record; all of the partial record portions combining to produce the predetermined saturation density of the full record; and each partial record portion including a variable contrast emulsion photo-responsive in a different spectral region from the other emulsions for independently controlling contrast in the preselected density range associated with the partial record portion.

10 Claims, 11 Drawing Figures



FIG. 2.

FIG. 1.



FIG. 3.



FIG. 10.



FIG. 11.



FIG. 4.



FIG. 5.



FIG. 6.



FIG. 7.



FIG. 8.



FIG. 9.

**MULTIPART PHOTOSENSITIVE ELEMENT  
WITH INDEPENDENT CONTRAST CONTROL OF  
CONSTITUENT PART RECORDS**

**FIELD OF INVENTION**

This invention relates to a multipart photosensitive element in which the contrast of each part record is independently controllable.

**BACKGROUND OF INVENTION**

Variable contrast black and white photosensitive elements exist in which the overall contrast can be varied using different wavelengths of light. This is done by using various sensitizers in conjunction with silver halides to enable one range of wavelengths of exposing radiation to produce high contrast, another low, and yet another intermediate, for example. While the overall contrast can be modified in this way, parts of the sensitometric curve cannot be independently altered.

**SUMMARY OF INVENTION**

It is an object of this invention to provide an improved, multipart photosensitive element having independent contrast control of constituent part records.

The invention features a multipart photosensitive element having a predetermined saturation density. There are at least two partial record portions for forming a full record. Each of the partial record portions controls a preselected density range of a full record. All the partial record portions combine to produce the predetermined saturation density of the full record. Each of the partial record portions includes a variable contrast emulsion photoresponsive in a different spectral region from the other emulsions, for independently controlling contrast in the preselected density range associated with the partial record portion.

The emulsions may be each in a separate layer or all in a single layer if their effective sensitivity ranges are substantially mutually exclusive, and may have complementary or non-complementary speeds. In the separate layer construction where the spectral regions of sensitivity of the emulsions may overlap, filter means may be inserted between these emulsions for attenuating radiation in the spectral range of one emulsion to which a second emulsion is also sensitive, in order to prevent that radiation from reaching the second emulsion.

The element may include a number of full records, as in a color film or color paper. One or more of these full records includes at least two partial record portions, as stated above. Each emulsion in each full color record is photoresponsive in different section of the spectral region associated with that color. If each of the emulsions in a particular full record have mutually exclusive or substantially mutually exclusive photosensitive spectral sections, then again they may be formed as a single layer. If not, they may be formed in separate layers with filter means between to split the light in that spectral region into separate sections to prevent exposure of subsequent emulsions by wavelengths which are meant to expose the previous emulsion.

**DISCLOSURE OF PREFERRED EMBODIMENT**

Other objects, features, and advantages will occur from the following description of preferred embodiments and the accompanying drawings, in which:

FIG. 1 is a diagram of a photosensitive element according to this invention;

FIG. 2 is an illustration of the family of varying contrast D-log E curves of the fast blue-sensitive emulsion of FIG. 1;

FIG. 3 is an illustration of the family of varying contrast D-log E curves of the slow red-sensitive emulsion of FIG. 1;

FIG. 4 is an illustration of the D-log E curves of FIG.

10 3, combined with the medium contrast curve of FIG. 2;

FIG. 5 is an illustration of the D-log E curves of FIG. 3, combined with the low contrast curve of FIG. 2;

FIG. 6 is an illustration of the D-log E curves of FIG. 3, combined with the high contrast curve of FIG. 2;

15 FIG. 7 is an illustration of the family of varying contrast D-log E curves of a fast blue-sensitive non-complementary speed emulsion shown in FIG. 1;

FIG. 8 is an illustration of the family of varying contrast D-log E curves of a slow red-sensitive non-complementary speed emulsion shown in FIG. 1;

20 FIG. 9 is an illustration of the D-log E curves of FIG. 8, combined with the medium contrast curve of FIG. 7;

FIG. 10 is a diagram of a photosensitive element according to this invention similar to FIG. 1, showing the use of the invention in conjunction with a negative working dye transfer system; and

25 FIG. 11 is a diagram of a photosensitive element according to this invention similar to FIG. 1, having three different full color records, one for the blue, one for the green, and one for the red records, each of which includes two partial records.

30 There is shown in FIG. 1 a photosensitive element 10; at least one full record 11 constituted by at least two or more part records 12 and 14; a support 16, baryta layer

35 18; and various spacer interlayers 20, 22, and 24, which may be of gelatin or of other similar materials used for making photographic emulsions; and a protective gelatin overcoat layer 26. Part record 12 includes emulsion

40 28, which may be formed of a fast blue-only sensitive silver halide, such as silver chloride, silver bromide, or silver chlorobromide, which have sensitivities in the range of approximately 360-410 nm, 375-470 nm, and some portion of the range from 360-470 nm, respectively.

45 A blue sensitizer such as 5-(2-ethyl-1(2)-benzothiazolylidene)-3-n-heptyl-rhodanine is included in emulsion 28 in the usual way to condition the emulsion a variable contrast material, for example using the technique explained in U.S. Pat. No. 2,384,598. If emulsion 28 is a silver chloride emulsion, then two sensitizers

50 must be added: one as above to condition it a variable contrast emulsion and another one to extend the high contrast of the region of inherent sensitivity further into the blue. A suitable sensitizer for this purpose would be 5-(2-ethyl-1(2)-benzothiazolylidene)-3-n-lauryl-2-thio-

55 2,4(3,5)-oxazoledione. Emulsion 28 typically has a saturation density between 0.6 and 1.2, with 0.7 to 1.0 being preferred.

Part record 14 includes emulsion 30, which may be formed of a slow, effectively red-light sensitive silver halide variable contrast emulsion. The same silver halides may be used, but of smaller average crystal size. Included with them may be two red sensitizers, one to extend the high contrast of the region of inherent sensitivity of the material into the red and a second to condition it as a variable contrast material. The first may be

60 5-[4-(2-ethyl-1(2)-benzoxazolylidene) butenylidene]-3-n-lauryl-rhodanine; and the second, which conditions emulsion 30 as a variable contrast material, may be

5-[4-(2-ethyl-1(2-benzothiazolylidene) butenylidene]-3-n-heptyl-rhodanine. Typically one of these sensitizers is in the shorter wavelength reds, while the other is in the longer wavelength reds.

If emulsion 30 has a sensitivity level in the blue region not substantially less than its level of sensitivity in the red spectral region, as in the case when these sensitizers are used for example, then a yellow, orange or red filter interlayer 32 may be placed between emulsions 28 and 30 in order to block blue light, essential to the functioning of emulsion 28, from reaching emulsion 30 where it would interfere with image formation. Interlayer 32 may be a filter mode using together the antihalation dyes of formula 8 and formula 5 of U.S. Pat. No. 3,544,325.

However, if the sensitivity of emulsion 30 to light outside of the red spectral region is sufficiently low so that no filter interlayer 32 is necessary, then the optional spacer interlayers 22 and 24 and filter interlayer 32 may be omitted; and in fact the two emulsions 28 and 30 may be formed as a single layer. For example, this may be done if instead of using the two sensitizers given above for emulsion 30, the sensitizer used in emulsion 30 to extend the high contrast of the region of inherent sensitivity into the red is 2,2',8-triethyl-4,4'-dichlorothiacarbocyanine bromide, and the sensitizer used in emulsion 30 to condition it for variable contrast is 3,3'-dimethyl-9-phenyl-4,5;4',5'-dibenzothiacarbocyanine chloride; the sensitizer(s) for emulsion 28 remain as given above.

A family of variable contrast curves 28a, FIG. 2, producible by emulsion 28, includes a high contrast curve 28aa, medium contrast curve 28ab, and low contrast curve 28ac. The exposure to obtain these curves is made in blue light. Their saturation densities are each 0.9. High contrast curve 28aa is made by exposure of emulsion 28 in short wavelengths of blue light only, for example such as by using a Kodak Polycontrast No. 4 filter. Exposure for medium contrast curve 28ab is made without a color filter so that both the shorter wavelength and longer wavelength of blue light to which emulsion 28 is sensitive is incident on element 10. Exposure to produce low contrast curve 28ac is produced by using predominately long wavelength blue light along with some short wavelength blue light as well, such as by using a Wratten 6 filter.

Similarly, the family of variable contrast curves 30a, FIG. 3, producible by emulsion 30, includes a high contrast curve 30aa, medium contrast curve 30ab, and low contrast curve 30ac, which are obtained by exposing element 10 to red light. Specifically, high contrast curve 30aa is produced by an exposure in short wavelength red light such as obtained using, for example, a Schott filter BG 18. Medium contrast curve 30ab is producible using a mixture of long and short wavelength red light in which no particular color filter is necessary, and low contrast curve 30ac is obtained using predominately long wavelength red light with some short wavelength red light as well, for example such as by using a Schott VG 13 filter. The saturation density reached by each of these curves is 1.4.

Thus each of the emulsions 28 and 30 may form a part record so that the part containing emulsion 28 may have any contrast range as illustrated by curve 28aa, 28ab, and 28ac; while the second part record of the full record formed by emulsion 30 may independently have any desired contrast range as indicated by curves 30aa, 30ab and 30ac.

Thus a full record provided by photosensitive element 10 utilizing part records formed of emulsions 28 and 30 may provide a medium contrast in the white and gray areas as indicated by medium contrast curve 28ab, FIG. 4, and either a high contrast, curve 30aa; medium contrast curve 30ab; or low contrast, curve 30ac, range of contrasts in the black area for a black and white reproduction. The photosensitive element 10 in this example has a preselected saturation density of 2.3, as a result of the accumulation of the 0.9 density of emulsion 28, and the 1.4 density of emulsion 30.

In FIG. 4 the toe of curves 30aa, 30ab and 30ac begin at about 0.78 log exposure, which coincides with the boundary density of 0.80 of medium contrast curve 28aa, and no adjustment is therefore necessary.

However, as shown in FIG. 5, when the low contrast range indicated by curve 28ac is chosen, the family of curves 30a must be shifted from their 0.78 log exposure position to a 1.1 log exposure position, in order that they properly meet the 0.8 boundary density of curve 28ac.

Similarly, as shown in FIG. 6, if the high contrast range indicated by curve 28aa is selected, the family of curves 30a must be shifted to the 0.54 log exposure point in order to properly match the boundary density of curve 28aa at 0.8. The shifting of the family of curves 30a is accomplished with filtration of the exposing light. Thus in FIG. 5 for matching the family of curves 30a with the low contrast curve 28ac, a red blocking filter such as a blue or cyan Kodak color correction filter, for example a CC40B or CC50C, is used to further slow down the response of the family of curves 30a, and move them from the 0.78 to 1.1 position of the log exposure range.

Conversely, with respect to FIG. 6, a blue blocking filter, such as for example a Kodak color correction filter CC30R, may be used to slow down the speed of the faster emulsion 28a.

Although thus far the invention has been described solely with respect to emulsions having complementary speeds; this is not required and this is not a necessary limitation of the invention, as they may be non-complementary as well. For example, emulsion 28 may have a saturation density of 2.0 so that it provides a family of curves 28'a, as shown in FIG. 7, and emulsion 30 may be formed to provide a family of curves 30'a, as shown in FIG. 8. Thus when combined to obtain the medium contrast range for the grays and whites as indicated by curve 28'ab, the preselected total density of the full record remains at 2.3, due to the surface reflection limit of 2.3 for a glossy paper, being discussed here; but the sum of the slopes remains constant until the reflection density of 2.3 is attained. This is due to the addition of curve 28'ab up to the 2.0 density point with whichever one of the family of curves 30'a is used. Curve 28'ab reaches saturation density after each of the accumulated density curves 30'aa, 30'ab, and 30'ac. This is shown in FIG. 9. Combination with the high and low contrast ranges indicated by curves 28'aa and 28'ac occurs in a similar fashion.

Although thus far the upper layer shown in FIG. 1 embodies the emulsion 28 fast blue-only light sensitive material and the lower layer embodies the emulsion 30 slow red-sensitive material, this is not necessarily a limitation of the invention. For example, the upper layer may be red sensitive and the lower layer blue sensitive; and the upper may be slow and the lower fast, with whatever filtration is necessary, if the spectral regions of sensitivity overlap.

The invention applies to positive or reversal elements as well as negative elements illustrated herein, and to both so-called wet process photosensitive elements and dry process photosensitive elements, including diffusion transfer process dye transfer systems such as Polaroid films. For example, in FIG. 10 there is shown a photosensitive element 10a which includes emulsion 28" and emulsion 30" with any necessary spacer interlayers 22, 24, and filtration 32, in conjunction with generally conventional materials used in such dye transfer systems; e.g., transparent support layer 50, polymeric acid layer 52, timing layer 54, image receiving layer 56, a layer 58 including a processing composition having opacifying dyes during processing and a white background material after processing is completed; and two black dye layers 60, 62, on an opaque support 64. A similar negative working system is explained in U.S. Pat. Nos. 3,443,939 and 3,751,406.

While thus far the invention has been illustrated by a photosensitive element depicting only one full record including but two part records, this is not a necessary limitation of the invention, there may be more than one full record and each full record may contain two or more such part records, provided that they are made generally, or at least effectively, mutually exclusive or substantially mutually exclusive as to their sensitivity. There may be as many different part records as there are desired number of distinct density ranges which are desired to have their contrast controlled. Thus a three-part full record could give separate control over the whites, grays, and blacks, while a five-part record might give control over the whites, light grays, midtone grays, dark grays and blacks.

One example is a color photosensitive element 10b, FIG. 11, using three full records, one for each of the primary image colors blue, green and red.

Each of the full records 60, 62, 64, includes at least two part records 12a, 14a; 12b, 14b; 12c, 14c. Part record 12a includes a fast blue emulsion 28d having effective sensitivity from about 400nm to 500 nm; and a slow 40 blue emulsion 30d is included in part record 14a having effective sensitivity from about 360 nm to 445 nm. Part record 12b includes a fast green emulsion 28e having effective sensitivity from about 390 nm to 560 nm, and slow green emulsion 30e is included in part record 14b 45 having effective sensitivity from about 400 nm to 600 nm. Part record 12c includes a fast red emulsion 28f having effective sensitivity from about 400 nm to 500 nm and from about 560 nm to 660 nm, and slow red emulsion 30f having effective sensitivity from about 380 50 nm to 715 nm is included in part record 14c. Emulsions 28d and 30d, 28e and 30e, 28f and 30f are sensitive in the areas of the spectrum associated with the color of the full record to which they contribute. If each pair of emulsions sensitive to the same general color are mutually exclusive, or substantially so, in their sensitivity within that region, then pairs may be made up as a monolayer instead of requiring a multilayer construction. The three fast emulsions should have the same effective photographic speed and whatever slope is chosen for them should be the same. This also applies to the slow emulsions although the selected slopes may be different from the slopes chosen for the fast emulsion.

Photosensitive element 10b, as shown, includes a blue splitting filter 70 for separating the blue spectral region for preventing, for example, light in the shorter wavelengths of blue to which emulsion 30d is sensitive from reaching and interfering with emulsion 28d.

As explained previously, added to each of these emulsions are the necessary sensitizers: one for the purpose of extending the high contrast of the region of inherent sensitivity into the appropriate spectral region; the other sensitizer for the purpose of conditioning the emulsion for variable contrast.

For example, the sensitizing dye used in emulsion 28d to extend the high contrast of the region of inherent sensitivity into the longer wavelengths of blue light may be 5-(2-ethyl-1(2)-benzothiazolylidene)-3-n-heptyl-rhodanine. The sensitizing dye used in emulsion 28d to condition it for variable contrast may be 3-carboxymethyl-1-(3-sulfopropyl)-oxa-2'-cyanine betanine.

The sensitizing dye used in emulsion 30d to condition it for variable contrast in the short wavelength spectral region of the blue may be 5-(2-ethyl-1(2)-benzothiazolylidene)-3-n-lauryl-2-thio-2,4(3,5)-oxazoledione. Its region of inherent sensitivity would be used for high contrast. This emulsion would be a silver chloride or a silver chlorobromide emulsion with only a small amount of silver bromide relative to silver chloride present to keep the region of inherent sensitivity to a portion of the range 360 nm to 420 nm.

The sensitizing dye used in emulsion 28e to extend the high contrast of the region of inherent sensitivity into the shorter wavelengths of green light may be 2-methyl-1'-ethylthia-2'-cyanine iodide. The sensitizing dye used in emulsion 28e to condition it for variable contrast may be 5-[(2-ethyl-1(2)-benzoxazolylidene)-ethylidene]-3-n-primaryheptyl-1-phenyl-2-thiohydantoin.

The sensitizing dye used in emulsion 30e to extend the high contrast of the region of inherent sensitivity into the longer wavelengths of green light may be 5-[(2-ethyl-1(2)-benzothiazolylidene)-ethylidene]-3-n-heptyl-1-phenyl-2-thiohydantoin. The sensitizing dye used in emulsion 30e to condition it for variable contrast may be 5,5',6,6'-tetrachloro-1,1'-diethyl-3,3'-bis ( $\gamma$ -sulfopropyl) benzimidazolocarbocyanine betaine sodium salt.

The sensitizing dye used in emulsion 28f to extend the high contrast of the region of inherent sensitivity into the shorter wavelengths of red light may be combination of sensitizing dye IH and supersensitizing dye IIB of U.S. Pat. No. 3,615,635. The structural formula for dye IH is given on column 4 of that patent while the structural formula for dye IIB is given on column 5 of that same patent. The sensitizing dye used to condition emulsion 28f for variable contrast may be dye 2 of U.S. Pat. No. 3,918,979. The structural formula for this dye is given on columns 3 and 4 of that patent.

The sensitizing dye used in emulsion 30f to extend the high contrast of the region of inherent sensitivity into the longer wavelengths of the red may be dye III-G of U.S. Pat. No. 3,907,575. [The structural formula for this dye is given on columns 15 and 16 of that patent.] The sensitizing dye used to condition emulsion 30f for variable contrast may be 3,3'-diethyl-9-(3-pyrrolyl)-4,5,4',5'-dibenzothiacarbocyanine bromide.

Photosensitive element 10b, as shown, includes a blue splitting filter 70 for separating the blue spectral region for preventing, for example, light in the shorter wavelengths of blue to which emulsion 30d is sensitive from reaching and interfering with emulsion 28d which is to record only in a longer wavelength blue light but is nonetheless sensitive to the shorter wavelength blue light. This may be a filter made using the antihalation dye of formula 1 of U.S. Pat. No. 3,687,670. The structural formula for this dye is given on column 3 of that patent. A filter can be made using this dye so that it

effectively blocks light in the wavelengths from about 380 nm to 455 nm. Between the first full record 60 and the second full record 62 is a yellow filter 72 which effectively blocks blue light which is no longer needed for the creation of the remaining part records of the full records 62 and 64, but to which those part records' emulsions may be sensitive. This may be a filter made using together the antihalation dye of formula 8 and the dye of formula 5, both of U.S. Pat. No. 3,544,325. The structural formulae for both dyes are given on column 4 of that patent. A filter can be made using these dyes so that it effectively blocks light in the wavelengths from about 380 nm to 500 nm. A green splitting filter 74 is provided between the green full record 62 emulsions 28e and 30e for the same purpose as the blue splitting filter 70, as explained above. This may be a filter made using the antihalation dye of formula 2 of U.S. Pat. No. 3,544,325. The structural formula for this dye is given on column 3 of that patent. A filter can be made using this dye so that it effectively blocks light in the wavelengths from about 380 nm to 550 nm.

Similarly, a magenta or red filter 76 is provided above red full record 64 in order to effectively block any blue or green light which is no longer necessary from reaching emulsions 28f and 30f, which might nonetheless be sensitive to that light. This may be a filter made using the antihalation dye of formula 3 of U.S. Pat. No. 3,471,293. The structural formula for this dye is given in column 2 of that patent. A filter can be made using this dye so that it effectively blocks light in the wavelengths from about 450 to 610 nm. A red splitting filter 78 is used between the red-sensitive emulsions 28f and 30f for the same purpose as the previous splitting filters were used between their respective part records. This may be a filter made using the antihalation dye of formula 4 of U.S. Pat. No. 3,471,293. The structural formula for this dye is given in column 3 of that patent. This dye strongly blocks light in the wavelengths from about 600 nm. to 665 nm. A filter can be made using this dye so that it effectively blocks light in wavelengths less than 665 nm. from exposing emulsion 30f. Various spacer interlayers 80 are used as necessary.

If instead of the sensitizer listed above for emulsion 28d for the purpose of conditioning it a variable contrast emulsion, Compound 3 of U.S. Pat. No. 3,847,613, whose structural formula is shown in column 2 of that patent, had been used together with 5-(2-ethyl-1(2)-benzothiazolylidene)-3-n-heptyl-rhodanine to extend the high contrast of the region of inherent sensitivity into the longer wavelengths of the blue, then emulsions 28d and 30d may be formed as a single layer. In this case, layer 70, the blue splitting filter, and the associated spacer interlayers 80 would be omitted. The reason this is possible is layer 28d with these two sensitizers has little effective sensitivity below 435 nm when compared with its sensitivity between 435 nm and 500 nm.

If instead of the sensitizer listed above for emulsion 30e for the purpose of extending the high contrast of the region of inherent sensitivity into the longer wavelengths of green light the following sensitizing dye had been used, then with no other changes in the sensitizers in emulsions 28e and 30e, emulsions 28e and 30e may be formed as a single layer. This replacement sensitizing dye may be 5,5',6,6'-tetrachloro-1,1',3,3'-tetraethylbenzimidazolocarbocyanine iodide. In this case, emulsion layer 30e has effective sensitivity only in two spectral regions: approximately 400-470 nm and 550 nm to 600 nm. Since filter layer 72 effectively blocks blue light

from reaching green full color record 62, emulsions 28e and 30e may be formed as a single layer. In this case, layer 74, the green splitting filter, and the associated spacer interlayers 80 would be omitted.

If instead of the sensitizer listed above for emulsion 30f that conditioned it for variable contrast the following sensitizing dye had been used, then with no other changes in the sensitizer and supersensitizer dyes used in emulsions 28f and 30f, emulsions 28f and 30f may be formed as a single layer. This replacement sensitizing dye is 5-[4-(2-ethyl-1(2)-benzothiazolylidene)butenylidene]-3-n-heptyl-rhodanine. In this case, emulsion layer 30f has effective sensitivity only in two spectral regions: approximately 370 nm to 470 nm and 650 nm to 715 nm. Since filter layer 72 effectively blocks blue light from reaching red full color record 64 as well, emulsions 28f and 30f may be formed as a single layer. In this case, layer 78, the red splitting filter, and the associated spacer interlayers 80 would be omitted.

Clearly, the use of the techniques of U.S. Pat. No. 2,384,598 has been illustrative and not limiting. Other techniques to make the constituent emulsions variable contrast emulsions can be used as well.

Other embodiments will occur to those skilled in the art and are within the following claims:

What is claimed is:

1. A multipart photosensitive element comprising: a support; a plurality of partial record portions carried on said support; all of said partial record portions together forming a full record; each of said partial record portions having a preselected density range of said full record and all of said partial record portion densities combined forming the total density range of said full record; each of said partial record portions including a variable contrast emulsion for varying the contrast of that partial record portion over its preselected density range; each of said variable contrast emulsions being photoresponsive in a different spectral region from the other emulsions in the other partial record portions for independently selectively varying the contrast in each of the partial record portions.

2. The multipart photosensitive element of claim 1 in which said emulsions are each in a separate layer.

3. The multipart photosensitive element of claim 1 in which said emulsions are all in a single layer.

4. The multipart photosensitive element of claim 1 in which said emulsions have complementary speeds.

5. The multipart photosensitive element of claim 1 in which said emulsions have non-complementary speeds.

6. The multipart photosensitive element of claim 2 in which the spectral regions of the sensitivity of a first of said emulsions overlaps with a second and said element further includes filter means between said emulsions for attenuating radiation in the spectral range of said first emulsion to which said second emulsion is also sensitive before that radiation reaches said second emulsion.

7. The multipart photosensitive element of claim 1 in which said element includes a number of different color full records each having said at least two partial record portions.

8. The multipart photosensitive element of claim 7 in which each emulsion in each different color full record is photoresponsive in a section of the spectral region associated with that color.

9. The multipart photosensitive element of claim 7 in which each of said emulsions of a said full record is in a separate layer, and said element further includes filter means disposed between said emulsions in a full color

record for attenuating radiation in the section of the spectral range of a first of said emulsions to which a subsequent emulsion is also sensitive before that radiation reaches that subsequent emulsion.

10. A multipart photosensitive element comprising: a support; first and second partial record portions carried on said support and together forming a full record; each of said partial record portions having a preselected density range of said full record and all of said partial record portion densities combined forming the total density range of said full record; each of said partial record portions including a variable contrast emulsion for varying the contrast of that partial record portion over its preselected density range; each of said variable

contrast emulsions being photoresponsive in a different spectral region from the other emulsions in the other partial record portions for independently selectively varying the contrast in each of the partial record portions; said first partial record portion emulsion including silver bromide and 5-(2-ethyl-1(2)-benzothiazoylidene)-3-n-heptyl-rhodanine as a sensitizer; and said second partial record portion emulsion including 10 silver bromide, 5[4-(2-ethyl-1(2)-benzoxazolylidene) butenylidene]-3-n-lauryl-rhodanine as a sensitizer and 5-[4-(2-ethyl-1(2)-benzothiazolylidene) butenylidene]-3-n-heptyl-rhodanine as a conditioner.

\* \* \* \* \*

15

20

25

30

35

40

45

50

55

60

65